

## UNITED STATES PATENT OFFICE

2,088,587

## TEXTILE THREADS AND FABRICS

Henry Dreyfus, London, England, and William Whitehead, Cumberland, Md., assignors to Celanese Corporation of America, a corporation of Delaware

No Drawing. Application February 5, 1936, Serial No. 62,476. In Great Britain February 9, 1934

7 Claims. (Cl. 117—2.1)

This invention relates to the manufacture of crêpe threads of filaments of cellulose acetate or other organic derivatives of cellulose and to the production of fabrics therefrom.

5 This application is a part continuation of our application S. No. 746,134, filed September 29, 1934.

Fabrics exhibiting crêpe effects have long been obtained by employing in their construction 10 highly twisted threads of natural silk in the gummed state, the crêpe effects appearing mainly when the fabrics so formed are subjected to an aqueous scouring treatment. The fabrics obtained by this process are highly valued on account of their pleasing appearance and handle. 15 The production of crêpe fabrics in an analogous manner by the use of crêpe threads of cellulose acetate has, however, been accompanied by difficulties. Generally, the crêpe effect obtained by simply applying to a cellulose acetate thread a 20 twist of the order of that commonly employed in connection with natural silk, weaving the twisted threads into a fabric and scouring the latter, is very unsubstantial and not comparable with that obtained with natural silk or regenerated cellulose artificial silk.

According to the present invention highly twisted crêpe threads of filaments of an organic derivative of cellulose are produced from threads 30 of filaments of an organic derivative of cellulose by crêpe twisting in at least two stages and steaming the threads during the insertion of twist in the final stage of twisting. It is of great advantage to have moisture present during the steaming.

35 Good results may be obtained by steaming at above 95° C. Steaming temperatures in the neighbourhood of 100° C. are especially to be recommended.

40 The invention is of especial value and will be more particularly described in connection with the production of crêpe threads of filaments of cellulose acetate.

The advantages of the new process may be obtained when the thread is steamed during the 45 insertion of twist both in the final stage of twisting and in an earlier stage or stages of twisting. In fact it is of great advantage to effect in the presence of steam any insertion of twist 50 beyond the point at which twisting would result in weakening of the thread if the said twisting were effected without the steaming. The precise degree of twist beyond which it is important to steam during twisting depends upon the total 55 denier of the thread and the number of its con-

stituent filaments. Generally at least the last half or two thirds of the total crêpe twist should be applied while steaming.

In this way it has been found possible to produce crêpe threads of filaments made from and consisting of cellulose acetate, which yield fabrics exhibiting remarkably good crêpe effects. Moreover, by this new process crêpe threads of cellulose acetate filaments may be produced which have an average strength much greater than that of crêpe threads produced by a simple twisting operation without the steam treatment during twisting. Further, apart from the great advantage of a stronger resultant thread the twisting operation itself is greatly facilitated in that twisting may satisfactorily be accomplished under conditions of twist and spindle speed which in the absence of the steaming would give rise to frequent thread breakage and render impossible the insertion of the desired twist or at least lead to a very weak and useless thread.

The threads may consist of substantially continuous filaments of cellulose acetate or they may contain discontinuous filaments of cellulose acetate, the length of which may vary within wide limits. For example the threads may be those spun from a mass of discontinuous filaments or those prepared in the manner described in British Patents Nos. 424,683, 424,752, 424,830 and 424,879. Again the crêpe threads may be made with filaments which contain water-insoluble compounds, whether compounds of pigment-like character in such form as materially to modify the lustre of the filaments (e. g. barium sulphate or titanium dioxide), or loading metal compounds, for example tin compounds.

In carrying out the new process the thread may be twisted by the rotation of a package from which it is being drawn off through a guide fixed substantially in line with the axis of rotation of the package, and thereafter wound on a bobbin or the like, the thread being passed, on its way from the guide to the bobbin, through steam under conditions such that moisture is present.

On the other hand, any other suitable crêpe twisting device may be employed. For example, a ring twister may be used when crêpe twisting thread consisting of discontinuous filaments.

The twisting spindle, the guide fixed in line with the axis of the spindle, and the steaming device should be so arranged that twist resulting from the rotation of the package is inserted while the thread is under the influence of the steam. For example, when twisting the thread

by the rotation of a package from which the thread is being drawn off, if the freedom of the thread to rotate within the balloon guide or other guide preceding or forming part of the steaming device is unduly restricted, e. g. by causing the 5 yarn to change direction materially at the guides, the insertion of twist while the thread is under the influence of the steam may be restricted to an undesirable extent, or substantially prevented, 10 and the resulting crêpe threads may not have the valuable properties which may otherwise be secured. Thus, when using a twisting device of the kind in which thread is drawn off from a rotating package, it is advantageous to arrange 15 that the path of the thread after leaving the balloon guide and through the steaming device, is substantially in line with the axis of the twisting spindle.

In the case of a ring twister, where twisting is 20 effected by the rotation of a package on to which the thread is being wound, the thread passing through steam on its way from the let-off device to the twisting spindle, a change of direction at the point where the thread leaves the steaming 25 device is of less importance as the thread remains under the influence of the steam for a short time after leaving the steaming device.

The phrase "twist is inserted while the thread is under the influence of steam" means that that 30 portion of the run of the thread in which twist is being inserted is either in the steam or still under the influence of the steam.

If desired, the above-mentioned twisting devices, in which the thread is drawn off from a rotating package, may be provided with a device 35 which restricts the ballooning of the yarn or the tendency of twist to run back to the package. As examples of such devices may be mentioned flyers and the floating ring device described in 40 U. S. Patent No. 1,784,581.

Steaming may conveniently be effected by allowing the thread to pass through a suitable chamber supplied with steam under such conditions that moisture is present.

45 Thus, a vertical twisting spindle of the type in which thread is drawn off upwardly over the end of a rotating package through a guide substantially in line with the axis of the spindle, may be provided with a small chamber situated vertically above the spindle. The chamber is provided with small holes, top and bottom, to permit passage of the thread, and also with a steam inlet. If desired, a single steam chamber may be arranged to serve a number of spindles, being 50 provided with inlet and outlet holes for the thread of each spindle. Such an apparatus may conveniently consist of a horizontal pipe mounted over a row of spindles and provided with eyes of porcelain, stainless steel, or other suitable material 55 at appropriate points on top and bottom for the entrance and exit of the threads. The diameter of the pipe is sufficient to afford the thread the requisite length of travel in the steam. Steam may be admitted to the pipe at one point or at 60 more than one point as may be necessary according to the length of the pipe, to secure sufficiently uniform conditions of steaming as between the threads from the different spindles.

At the point at which the thread from the 70 twisting spindle enters the steaming device, it is advantageous to arrange a free escape of steam on to the thread as it is drawn off from the spindle. A shield, for example in the form of a funnel, may, if desired, be fitted around the 75 thread approaching the steaming device in order

to maintain an atmosphere of steam around the thread.

The presence of the desired moisture may be assured by arranging for the condensation of steam. Dry steam may be passed through water 5 so as to saturate the steam and the requisite moisture produced by cooling in the steaming device.

Another method of ensuring the presence of moisture is to wet the thread with water; for 10 example the bobbins of thread may be wetted before the twisting operation or better, water may be applied to the thread, by means of a wick or other device, after the thread leaves the spindle and prior to its entering the steaming device. 15 The water may contain a substance which facilitates wetting of the thread by water.

Steam at about atmospheric pressure, e. g. slightly above atmospheric pressure, is most conveniently employed. If desired, however, the 20 steaming may be effected with steam at higher pressures, e. g. steam at 10-25 lbs. per square inch.

A steaming treatment of relatively short duration such as may be secured by passing the yarn 25 at a speed of from 2 to 10 metres per minute through 3" of steam has been found to give satisfactory results. Lengthier treatments may, however, be employed, for example the yarn may be passed at the said speeds through 6 to 12" of 30 steam or more.

The cellulose acetate filaments of the threads very readily undergo stretching when the threads are twisted under the influence of the steam and moisture. The amount of stretch may be measured by comparing the original thread denier with the final thread denier (after untwisting). The denier of the resultant thread is, in general, owing to imparted stretch, less and even substantially less than if the steam treatment is omitted. 40 The stretch imparted to the filaments of the threads during the twisting operation may for example be of the order of 5-25% of their original length, and particularly 10-20%. The degree of stretching of the filaments of the thread may be 45 such that the final denier of the crêpe twisted thread is not much in excess of or is even the same or less than the denier of the thread prior to crêpe twisting. For example the stretch may be such that the denier of the crêpe twisted 50 thread is from 95 to 115%, particularly 100 to 110% of that of the thread before crêpe twisting, especially in the case of threads having an original denier of 150 or less. Good crêpe fabrics may however be obtained when the final denier 55 is still greater, for example up to 120% of that of the thread before twisting when threads having a denier about 200 are employed.

The total twist inserted in accordance with the new process may vary within wide limits. The 60 new process possesses the feature that it enables a very high degree of twist to be inserted without the great weakening of the thread such as is generally experienced when a cellulose acetate thread is twisted without the steaming to the 65 degree necessary in a crêpe thread. The process, moreover, permits the insertion of twists which are impossible of attainment without the steaming owing to breakage of the thread. This is important since it enables crêpe fabrics to be 70 produced having very pronounced crêpe effects. The crêpe figure can be regulated according to requirements. The total twist desirable in any particular case depends upon the denier of the thread. For example with threads of 165 denier 75

twist of about 70 to 75 turns per inch is desirable, and with threads of 115 denier twist of about 85 to 90 turns per inch. With these indications it is a simple matter to determine the desirable twists for threads of other deniers. The denier numbers given are those of the threads after crêpe twisting.

The twist may be divided between the twisting stages in various proportions. Twist inserted in the absence of steam should not be of such degree as to damage the thread. To this end, as indicated previously, twisting in the absence of steam should not be effected where the twist inserted is sufficient to result in substantial weakening of the thread.

A particularly convenient method of working is to apply about one sixth to one quarter or one half of the total crêpe twist without steam, say up to 10 or 15-25 or even up to 30 or 40 turns per inch, and then to complete the crêpe twist in the presence of steam and moisture.

As indicated above, by the new process highly twisted threads of cellulose acetate filaments may be produced which are of high crêping power. In these threads the filaments are extremely closely packed, a feature to which their good crêping power may be attributed. For example, the filaments may be so closely packed that the apparent specific gravity of the thread as determined from the diameter and the denier is more than 85%, e. g. 85 to 90% of the actual specific gravity of the filaments, and that distortion of the cross-section of at least some of the filaments has occurred during the process of twisting. The filaments of the thread, however, are not stuck together and can be separated upon untwisting. Moreover, these cellulose acetate crêpe threads are smooth and cylindrical as opposed to the rough feel and helical form of a cellulose acetate thread or a viscose thread which has been crêpe twisted in the ordinary way. Further, in comparison with these latter threads, the smooth cylindrical cellulose acetate crêpe threads exhibit much less tendency to snarl or kink.

While the new process enables production of threads which yield satisfactory crêpe effects without a special treatment, other than the twisting and steaming treatment characteristic of the process, other devices and treatments may, if desired, be employed further to improve the properties of the crêpe threads and/or fabrics produced therefrom. For example the crêpe threads may be sized at any suitable stage of their manufacture, for example in the course of winding on to the bobbin from which twisting is effected. In this connection, particular mention may be made of sizing materials selected in accordance with the considerations laid down in U. S. Patent No. 2,007,182. For example a casein, egg-albumen, or other size which is not very readily removed by aqueous treatments may be employed. Another size which may be employed is a drying oil, if desired one which has been partially oxidized, e. g. boiled or blown linseed oil.

The highly twisted crêpe threads may be incorporated in the fabrics in various ways, for example the weft alone may be wholly or partially composed of such threads or the warp may also contain them. Valuable fabrics may be produced by employing warp threads of relatively low twist and in the weft both crêpe threads having a left-hand twist and crêpe threads having a right-hand twist, pairs of threads of left-hand

twist alternating with pairs of threads of right-hand twist.

If desired the cellulose acetate crêpe threads may be associated in the fabrics with highly twisted crêpe threads of other materials, e. g. of natural silk or regenerated cellulose, or with highly twisted threads produced by other processes. Where the fabrics contain threads of low twist these may be wholly of cellulose acetate or wholly or in part of other materials, e. g. natural silk or regenerated cellulose.

Fabrics containing highly twisted crêpe threads prepared in accordance with the invention may subsequently be given a hot aqueous treatment, for example in the manner commonly adopted in connection with fabrics comprising highly twisted yarns of natural silk. Enhanced crêpe effects may be obtained by means of hot aqueous treatments at or near the boiling point.

Instead of threads of filaments made from and consisting of cellulose acetate, threads of filaments of other organic derivatives of cellulose may be crêpe twisted in a similar manner. As examples of such other organic derivatives of cellulose may be mentioned cellulose formate, propionate or butyrate, or other organic esters of cellulose, and methyl, ethyl, benzyl and other ethers of cellulose.

Having described our invention what we desire to secure by Letters Patent is:—

1. Process for the production of a highly twisted crêpe thread of filaments of an organic derivative of cellulose, which comprises crêpe twisting a thread of filaments of an organic derivative of cellulose in at least two stages and inserting twist in at least the final stage while the thread is subjected to the action of steam.

2. Process for the production of a highly twisted crêpe thread of filaments of an organic derivative of cellulose, which comprises crêpe twisting a thread of filaments of an organic derivative of cellulose in at least two stages and inserting twist in at least the final stage while the thread is subjected to the action of moist steam.

3. Process for the production of a highly twisted crêpe thread of cellulose acetate filaments, which comprises crêpe twisting a thread of cellulose acetate filaments in at least two stages and inserting twist in at least the final stage while the thread is subjected to the action of steam.

4. Process for the production of a highly twisted crêpe thread of cellulose acetate filaments, which comprises crêpe twisting a thread of cellulose acetate filaments in at least two stages, of which the final stage involves insertion of at least half of the total crêpe twist, and inserting twist in the final stage while the thread is being steamed.

5. Process for the production of a highly twisted crêpe thread of cellulose acetate filaments, which comprises crêpe twisting a thread of cellulose acetate filaments in at least two stages, and inserting twist in at least the final stage while the thread is being steamed with moist steam, the filaments of the thread being stretched by 5 to 25% of their original length.

6. Process for the production of a highly twisted crêpe thread of cellulose acetate filaments, which comprises crêpe twisting a thread of cellulose acetate filaments in at least two stages, and during the final stage of twisting steaming the thread by passing it through a substantially closed chamber maintained full of steam.

steam under conditions such that moisture is present, so that twist is inserted as the thread passes through the steaming chamber, the final stage of twisting being effected by the rotation of a package from which the thread is being drawn.

5. 7. Process for the production of a highly twisted crêpe thread of cellulose acetate filaments, which comprises crêpe twisting a thread of cellulose acetate filaments in at least two stages, and during the final stage of twisting

steaming the thread by passing it through a substantially closed chamber maintained full of steam at substantially 100° C. under conditions such that moisture is present, so that twist is inserted as the thread passes through the steaming chamber, the final stage of twisting being effected by the rotation of a package from which the thread is being drawn.

5

HENRY DREYFUS.

WILLIAM WHITEHEAD.

10

## CERTIFICATE OF CORRECTION.

Patent No. 2,088,587.

August 3, 1937.

HENRY DREYFUS, ET AL.

It is hereby certified that error appears in the printed specification of the above numbered patent requiring correction as follows: Page 3, second column, line 75, claim 6, and page 4, second column, line 1-2, claim 7, strike out the words "substantially closed"; and that the said Letters Patent should be read with these corrections therein that the same may conform to the record of the case in the Patent Office.

Signed and sealed this 5th day of October, A. D. 1937.

Henry Van Arsdale

(Seal)

Acting Commissioner of Patents.

steam under conditions such that moisture is present, so that twist is inserted as the thread passes through the steaming chamber, the final stage of twisting being effected by the rotation of a package from which the thread is being drawn.

5. 7. Process for the production of a highly twisted crêpe thread of cellulose acetate filaments, which comprises crêpe twisting a thread of cellulose acetate filaments in at least two stages, and during the final stage of twisting

steaming the thread by passing it through a substantially closed chamber maintained full of steam at substantially 100° C. under conditions such that moisture is present, so that twist is inserted as the thread passes through the steaming chamber, the final stage of twisting being effected by the rotation of a package from which the thread is being drawn.

5

HENRY DREYFUS.

WILLIAM WHITEHEAD.

10

## CERTIFICATE OF CORRECTION.

Patent No. 2,088,587.

August 3, 1937.

HENRY DREYFUS, ET AL.

It is hereby certified that error appears in the printed specification of the above numbered patent requiring correction as follows: Page 3, second column, line 75, claim 6, and page 4, second column, line 1-2, claim 7, strike out the words "substantially closed"; and that the said Letters Patent should be read with these corrections therein that the same may conform to the record of the case in the Patent Office.

Signed and sealed this 5th day of October, A. D. 1937.

Henry Van Arsdale

(Seal)

Acting Commissioner of Patents.

CERTIFICATE OF CORRECTION.

Patent No. 2,088,587.

August 3, 1937.

HENRY DREYFUS, ET AL.

It is hereby certified that error appears in the printed specification of the above numbered patent requiring correction as follows: Page 3, second column, line 75, claim 6, and page 4, second column, line 1-2, claim 7, strike out the words "substantially closed"; and that the said Letters Patent should be read with these corrections therein that the same may conform to the record of the case in the Patent Office.

Signed and sealed this 5th day of October, A. D. 1937.

Henry Van Arsdale

(Seal)

Acting Commissioner of Patents.